

July 22, 1924.

1,502,514

D. B. MITCHELL ET AL

MANUFACTURE OF WATERPROOF PAINT

Filed May 28, 1923



David B. Mitchell,  
George J. Mitchell,

by Bright & Bailey,  
Attorneys

Patented July 22, 1924.

1,502,514

# UNITED STATES PATENT OFFICE.

DAVID B. MITCHELL AND GEORGE J. MITCHELL, OF LOUISVILLE, KENTUCKY

## MANUFACTURE OF WATERPROOF PAINT.

Application filed May 28, 1923. Serial No. 641,944.

To all whom it may concern:

Be it known that we, DAVID B. MITCHELL and GEORGE J. MITCHELL, citizens of the United States, and residents of Louisville, 5 in the county of Jefferson and State of Kentucky, have invented certain new and useful Improvements in the Manufacture of Waterproof Paint, of which the following is a specification.

10 Our invention relates to the manufacture of waterproof paint.

In carrying our invention into practice, it has been our purpose to produce novel and efficient bases and vehicles for waterproof paint of such nature that we are enabled to completely utilize, in the manufacture thereof, commercial tire rubber having fabric vulcanized therein, as exemplified by old discarded automobile tires.

20 It is also our purpose to provide a novel and advantageous process for rendering the rubber and fabric of discarded automobile tires into such form that their elements can be entirely utilized to great advantage in 25 the production of our improved paint bases and which process will also provide other ingredients for use as a vehicle in our improved paint or independently thereof.

Furthermore, it is our purpose to provide 30 a novel and efficient apparatus for carrying out the aforementioned process in an economical manner.

In describing our invention in detail we will make reference to the accompanying 35 drawing wherein is illustrated a diagrammatic view of our improved apparatus. Said apparatus is shown as comprising a pair of air tight cookers A and B which are mounted upon and in operative relation 40 to suitable furnaces 2 and 11, respectively, whereby they may be maintained at a desired temperature. The furnace 2 is provided with a smoke pipe 7 having a damper 7' and this smoke pipe is connected between 45 the damper and furnace with the interior of the furnace 11 by a pipe 8 having a damper 8'. As a result of this construction it will be apparent that by closing the damper 7' and opening the damper 8', the heat generated 50 in the furnace 2 may be transmitted to the furnace 11, in lieu of directly firing the latter. Access to the interior of the cookers A and B is had through manholes in the top thereof which are closed by detachable covers 4 and 12 respectively. The cooker A carries therein a horizontal per-

forated partition 3 spaced from the bottom of the cooker. This partition is of a suitable folding type, whereby it may be applied and removed through the manhole closed by the 60 cover 4. A corresponding partition 10 is provided in the cooker B. A valved pipe 5 connects the top of the interior of the cooker A with the interior of the cooker B, the connection of said pipe with the 65 cooker B being at a point between the bottom of the cooker and the partition 10. Our apparatus further embodies condensers C and D of well known construction, the upper end of the condenser C being connected with the top of the interior of the cooker B by a valved pipe 14, while the condenser C is connected adjacent its lower end with the condenser D by a valved pipe 22. The condensers C and D are further 70 provided with condensate drain valves 21 and 28 respectively for a purpose that will 75 presently appear.

Our apparatus previously described is particularly adapted for carrying into effect our improved process whereby we are enabled to render fabric carrying commercial tire rubber into such form as to provide essential ingredients for our waterproof paint base, the provision of such ingredients completely utilizing every portion of such fabric carrying commercial tire rubber. In carrying our process into effect through the medium of said apparatus we remove the cover 4 of cooker A and in 80 turn remove the partition 3. We then place a charge of rosin on the bottom of said cooker and replace the partition. On this partition we place a charge of fabric carrying commercial tire rubber, such as old 85 discarded automobile tires, and restore the cover 4. The charges placed in the cooker are in the proportion of substantially 30% rosin and 70% fabric carrying commercial tire rubber. We then remove the cover 12 90 of cooker B and place a suitable charge of said rubber on partition 10. The cover 12 is then replaced, the damper 7' closed and 95 damper 8' opened. The furnace 2 is then fired to maintain the temperature of the 100 cooker A at substantially 450° F. Under those conditions, the charge of rosin will be progressively vaporized and such vapor will pass through the perforations of partition 3 and contact with the rubber and 105 fabric, which contact of heated vapor with said material will progressively render the 110

rubber fluent and so act on the fabric as to cause the latter to completely disintegrate when subjected to slight pressure or in other words, the fabric becomes a mere rubber impregnated pulp with no appreciable body texture. As the rubber becomes fluent it flows through the perforations of the partition 3 into the rosin therebeneath and this mixture is drawn off through valve 6. 5

10 The rubber impregnated fabric remaining on partition 3 is then removed, crushed and ground and the resulting product incorporated in the mixture of rosin and rubber previously withdrawn through valve 6 to 15 produce our improved base for waterproof paint of a coarse grade. While the cooking operation in cooker A is proceeding, it will be apparent that the cooker B will be suitably heated by the products of combustion 20 passing through pipe A from furnace 2. Likewise the rosin vapor which passes through the material on partition 3 in cooker A will in turn enter the cooker B below partition 10 by way of pipe 5 and act 25 on the material carried by the partition 10 to render the rubber fluent and destroy the body texture of the rubber permeated fabric. The rubber rendered fluent on the partition 10 will flow into the lower portion of cooker 30 B and is then drawn off through valve 15. The rubber permeated fabric remaining on partition 10 is then removed, ground and crushed, and mixed with the fluent rubber drawn off at valve 15 to provide a more 35 refined base for waterproof paint. The refinement of this base over the corresponding base obtained from cooker A is due to the fact that the rendered material is not directly mixed with the rosin and is further removed from the cooking charge of 40 the latter, and therefore, such base does not contain the heavy, sticky, resinous substance present in the base obtained from cooker A.

45 Our process and apparatus further provides a suitable and desirable vehicle for the paint bases previously described by converting the vapor of the rosin into an oil through the medium of condensation. We 50 accomplish this end by conveying the vapor from cooker B to condenser C by means of pipe 14. That portion of the vapor which is condensed by the condenser C is drawn off at valve 21, while that portion which is 55 not so condensed is carried to condenser D by way of pipe 22 where it is in turn condensed and forms a lighter oil than that produced by condenser C. Our improved paint bases can be mixed with either of 60 these oils to provide the finished paint or they can be associated with any other desirable paint vehicle. Likewise the oils obtained at condensers C and D can be associated with any desired paint bases or used 65 independently. For instance, we have dis-

covered that the oil obtained at condenser C can be employed effectively for polishing, staining, etc., while the oil obtained at condenser D, which is lighter, can be used for thinning or as a drier for paints. Thus it 70 will be seen that all material employed in our process is utilized without loss or waste and corresponding economy in the manufacture of our improved paint thereby had, which economy is further emphasized by 75 the fact that most of the material utilized in such manufacture is now generally recognized as practically worthless. We also desire to call attention to the fact that the quality of finished paints having our improved bases are greatly enhanced by reason of the presence of ground and crushed fabric therein of the type heretofore described, which element we have found acts as a most efficient binder when the paint is 80 applied.

We claim:—

1. The process of producing a base for waterproof paint which consists in rendering commercial tire rubber fluent by contacting the vapor of heated rosin therewith and then mixing the fluent rubber with heated rosin. 90

2. The process of producing a base for waterproof paint which consists in rendering commercial tire rubber fluent by contacting the vapor of heated rosin therewith and allowing the fluent rubber as it forms to flow into the heated rosin from which said vapor emanated. 95

3. The process of producing a base for waterproof paint which consists in contacting the vapor of heated rosin with commercial tire rubber having fabric vulcanized therein to render the rubber fluent, mixing the fluent rubber with heated rosin, then crushing and grinding the remaining fabric and residue of rubber in association therewith and mixing the same with the previously obtained mixture of rubber and 105 rosin. 110

4. The process of producing a base for waterproof paint which consists in contacting the vapor of heated rosin with commercial tire rubber having fabric vulcanized 115 therein to render the rubber fluent, draining off the resultant fluent rubber as it forms into the heated rosin from which said vapor emanated, then crushing and grinding the remaining fabric and the residue of 120 rubber in association therewith and mixing the same with the previously obtained mixture of rubber and rosin. 125

5. The process of disintegrating commercial tire rubber having fabric vulcanized 130 therein which consists in contacting therewith the vapor of heated rosin to render the rubber fluent and separating the fluent rubber from the fabric.

6. The process of producing a base for 130

waterproof paint which consists in confining a charge of commercial tire rubber above a charge of rosin in an air tight cooker, heating the rosin to a temperature sufficiently elevated to cause vapor to emanate therefrom, contacting this vapor with the rubber to render the latter fluent, draining the fluent rubber as it forms into the heated charge of rosin and then draining off the mixture of rubber and rosin.

7. The process of producing a base for waterproof paint which consists in confining a charge of commercial tire rubber, having fabric vulcanized therein, above a charge of rosin in an air tight cooker, heating the rosin to a temperature sufficiently elevated to cause vapor to emanate therefrom, contacting this vapor with the rubber and fabric to render the rubber fluent, draining the fluent rubber as it forms into the heated charge of rosin, drawing off the mixture of rubber and rosin, removing and crushing and grinding the fabric, and then mixing the ground and crushed fabric with the mixture of rubber and rosin.

8. The process of producing a base for waterproof paint which consists in confining a charge of commercial tire rubber, having fabric vulcanized therein, above a charge of rosin in an air tight cooker, maintaining the temperature of the rosin at substantially 450° F. until the resulting vapor from the rosin contacting with the rubber and fabric renders the former fluent, draining the fluent rubber as it forms into the heated charge of rosin, drawing off the mixture of rubber and rosin, removing and crushing and grinding the fabric, and then mixing the crushed and ground fabric with the mixture of rubber and rosin.

9. The process of producing a base for waterproof paint which consists in confining in an air tight cooker a charge of commercial tire rubber, having fabric vulcanized therein, above a charge of rosin, in the proportion of 70% rubber and fabric and 30% rosin, heating the rosin to a temperature sufficiently elevated to cause vapor to emanate therefrom, contacting this vapor with the rubber and fabric to render the former fluent, draining the fluent rubber as

it forms into the heated charge of rosin, drawing off the mixture of rubber and rosin, removing and crushing and grinding the fabric and then mixing the crushed and ground fabric with the mixture of rubber and rosin.

10. The process of producing a base and vehicle constituents of waterproof paint which consists in contacting the vapor of heated rosin with commercial tire rubber having fabric vulcanized therein to render said rubber fluent, condensing the vapor from the rosin which passes through the rubber to form the paint vehicle, draining the fluent rubber from the fabric, crushing and grinding the fabric, and then mixing the crushed and ground fabric with the previously drained fluent rubber to form the paint base.

11. The process of producing a base for waterproof paint which consists in contacting the vapor of heated rosin with commercial tire rubber, having fabric vulcanized therein, to render the rubber fluent, draining the fluent rubber from the fabric, crushing and grinding the fabric and then mixing the crushed and ground fabric with the previously drained fluent rubber.

12. A waterproof paint formed of a base of rubber, fabric and rosin, and a vehicle constituted by the condensate of the vapor of heated rosin after the latter has passed through a mass of rubber.

13. The process of producing a base for waterproof paint which consists in rendering rubber fluent by contact with the vapor of heated rosin therewith and then mixing the fluent rubber with heated rosin.

14. The process of producing a base for waterproof paint which consists in contacting the vapor of heated rosin with rubber having fabric vulcanized therein to render the rubber fluent, draining the fluent rubber from the fabric, crushing and grinding the fabric, and then mixing the crushed and ground fabric with the previously drained fluent rubber.

In testimony whereof we hereunto affix our signatures.

DAVID B. MITCHELL.  
GEORGE J. MITCHELL.